

1,038,271.

G. H. BENJAMIN.  
METHOD OF TREATING METAL INGOTS.  
APPLICATION FILED FEB. 24, 1911.

Patented Sept. 10, 1912.

FIG.1.



FIG.2.



FIG.3.



FIG.4.



FIG.5.



WITNESSES:

Charles W. Dunn  
Helen E. Kollack

G. H. Benjamin

# UNITED STATES PATENT OFFICE.

GEOEGE HILLARD BENJAMIN, OF NEW YORK, N. Y

## METHOD OF TREATING METAL INGOTS.

1,038,271.

Specification of Letters Patent. Patented Sept. 10, 1912.

Application filed February 24, 1911. Serial No. 610,526.

To all whom it may concern:

Be it known that I, GEORGE HILLARD BENJAMIN, a citizen of the United States, residing in the city, county, and State of New York, have invented certain new and useful Improvements in the Method of Treating Metal Ingots, of which the following is a specification.

As is well known, metal ingots during the act of cooling, are subjected to the action of two forces, *i. e.*, (1) contraction, with the resultant formation of depressions or pipe in the body of the ingot, and (2) segregation, due to the difference in specific gravity of the materials forming the ingot, with the result of unequal distribution of materials throughout the ingot.

The object of my invention is to overcome the above stated objections.

To carry my invention into effect, I may use apparatus such as disclosed in the accompanying drawings. I wish it understood, however, that these drawings are in a sense diagrammatic and merely intended to illustrate such apparatus as may be used, without in any wise intending to confine myself to the specific apparatus disclosed.

In the drawings, Figures 1 and 2 are respectively horizontal and vertical sections of a mold provided with heating means. Fig. 3 is a horizontal plan view of a mold provided with cooling means. Fig. 4 is a vertical section of an apparatus in which an ingot may be subjected to lateral pressure along a portion of its length and rotated, and Fig. 5 is a partial plan view and horizontal section of Fig. 4.

In all of the figures an ingot is illustrated as in position.

As a preliminary step in the production of the ingot, I pour the molten metal A into a mold B, so constructed that at least one side of the mold shall have a higher temperature than the other sides of the mold. This difference in temperature may be obtained by heating one side of the mold, or one half of the mold, by heating apparatus C, C' (Figs. 1 and 2), or by chilling three sides of the mold by a cooling apparatus D, (Fig. 3), the particular design of heating or cooling apparatus being immaterial, so long as that used will accomplish the purpose desired. By casting the ingot in a mold having one side of higher temperature than the other sides, one side of the ingot

will retain a higher temperature than the other sides and as shrinkage takes place in the cooling of the ingot, the soft metal upon the heated side of the ingot will accommodate for such shrinkage and the usual cupping or the formation of pipe will be prevented. After the ingot is cool enough to handle, it is lifted from the mold, placed upon a carriage E, and inserted between pressure plates F—G, mounted upon shafts H, carried in suitable bearings I. The plate G is made adjustable to and from the ingot through the instrumentality of a hydraulic piston J. The plate F is divided into two portions, one portion of which is fixed and the other portion K, made adjustable to and from the ingot A, by means of the hydraulic piston L. The purpose in using adjustable portion K of the plate F, is to provide means for compressing a portion of the soft side of the ingot, during the time shrinkage is taking place and the ingot cooling. Simultaneously with the exertion of pressure by the portion K of the plate F, the ingot is slowly rotated. The effect of the rotation is to overcome the tendency to segregation of the materials forming the ingot under the action of gravity, and this is aided by the lateral pressure along a portion of its length exerted through the portion K of the plate F.

I am aware that it has heretofore been proposed to rotate the ingot during the time that the ingot is cooling, and also to exert lateral pressure along the whole side of the ingot, and such I do not claim as my invention.

What I claim as my invention is:

1. A step in the method of treating ingots which consists in casting the metal into a mold and maintaining the temperature of one side of the mold relatively higher than that of the other sides and bottom of the mold during the whole time that the ingot is cooling.

2. A step in the method of treating ingots which consists in rotating the ingot after casting, and simultaneously subjecting the ingot to lateral pressure along a portion of its length exerted against the warm side of the ingot.

3. The method of treating ingots which consists in first casting it in such manner that one side of the ingot shall be warmer than the other sides, and subsequently sub-

jecting the ingot to rotation and to lateral pressure along a portion of its length exerted against the warm side of the ingot.

4. The method of treating ingots which 5 consists in casting it into a mold provided with means whereby one side of the mold shall be warmer than the other sides, then withdrawing the ingot, rotating the ingot and subjecting the warmer side of the ingot 10 to the action of lateral pressure along a portion of its length.

5. The method of treating ingots which 15 consists in casting the metal into a mold, and then regulating the temperature of the sides and bottom of the mold to have that of one side relatively higher than that of the other sides and bottom, whereby all the shrinkage of the ingot will take place from without inward and at one side.

20 6. The method of treating ingots which consists in casting the metal into a mold, regulating the temperature of the sides and

bottom of the mold to have that of one side maintained at a different temperature than that of the other sides and bottom, whereby 25 the shrinkage of the ingot will take place from without inward at one side, and then subjecting the ingot to lateral pressure transmitted from the side at which the shrinkage has taken place.

30 7. The method of treating ingots which consists in casting the metal into a mold, then subjecting the molten metal in the mold to a definite maintained temperature along three sides and the bottom of the 35 mold, and to a different maintained degree of temperature along one side.

In testimony whereof, I affix my signature, in the presence of two witnesses.

GEORGE HILLARD BENJAMIN.

Witnesses:

H. E. KOELSCH,  
CHARLES W. DUNN.